

Feb. 2, 1960

H. JAFFE ET AL

2,923,605

## METHOD OF GROWING QUARTZ SINGLE CRYSTALS

Filed Sept. 29, 1954

3 Sheets-Sheet 1



FIG. I



FIG. 2

*INVENTORS*  
HANS JAFFE  
THADDEUS J. TUROBINSKI

BY William J. Flynn  
ATTORNEY

Feb. 2, 1960

H. JAFFE ET AL.

2,923,605

## METHOD OF GROWING QUARTZ SINGLE CRYSTALS

Filed Sept. 29, 1954

3 Sheets-Sheet 2



*INVENTORS*

BY William J. Flynn  
ATTORNEY

Feb. 2, 1960

H. JAFFE ET AL

2,923,605

METHOD OF GROWING QUARTZ SINGLE CRYSTALS

Filed Sept. 29, 1954

3 Sheets-Sheet 3



FIG. 4



FIG. 5

INVENTORS'

HANS JAFFE  
THADDEUS J. TUROBINSKI

BY *William J. Flynn*  
ATTORNEY

## 1

2,923,605

**METHOD OF GROWING QUARTZ SINGLE CRYSTALS**

Hans Jaffe and Thaddeus J. Turobinski, Cleveland Heights, Ohio, assignors to Clevite Corporation, Cleveland, Ohio, a corporation of Ohio.

Application September 29, 1954, Serial No. 459,052

8 Claims. (Cl. 23—301)

This invention relates to the growing of artificial quartz single crystals.

Crystal plates of quartz have for many years been used extensively as frequency determining elements in radio frequency oscillators, electrical filters, and the like. In consequence of the continuing demand for such crystal plates, considerable advances have been made in recent years in the synthesis of large single crystals of quartz from which such crystal plates may be fabricated. Illustrative of such advances are the apparatus and method described and claimed in U.S. Letters Patent 2,675,303 to Andrew R. Sobek and Danforth R. Hale, assigned to the same assignee as the present invention. In accordance with the general procedure of this patent, successful synthesis of single crystals of quartz has been obtained by exposing a quartz crystal seed under conditions of elevated temperature and pressure to an aqueous medium containing substantial quantities of an alkali metal carbonate, such as sodium carbonate or sodium bicarbonate. The aqueous medium is maintained in contact with a supply material of crystalline quartz and crystal growth takes place by the transfer of silica from the supply material to the quartz seed. Other methods have also been employed with success in which the quartz seed is exposed to other suitable predetermined chemical and physical environments which promote crystalline growth on the seed to produce a quartz crystal bar from which crystal plates may be fabricated.

Experience in the synthesis of single crystals of quartz in the various chemical and physical environments in which successful growth has been achieved has demonstrated that quartz is one of the types of crystals which usually grow elongated in one direction, in the case of quartz, along the Z crystal axis. The fully grown quartz crystal, either synthetic or natural, between its ends tends to be in the shape of an elongated prism bounded by a set of six faces, known as the primary prism faces, which extend in the direction of natural elongation of the crystal. At either end the crystal is terminated primarily by three intersecting faces, known as the major rhombohedral faces, which produce tapered end caps on the crystal. If a quartz crystal seed body of any desired size and shape is permitted to grow indefinitely, it will eventually develop into a crystal bounded at the sides by the primary prism faces and at either end by the major rhombohedral faces. Little or no crystal growth takes place on these faces after they have formed fully in the chemical and physical environments used successfully in growing quartz crystals.

One of the most important aspects of quartz synthesis is to obtain the maximum yield, i.e., the greatest amount of material usable for crystal plates, from a given plant in a given time. Heretofore, it has been necessary to employ relatively large quartz seed plates and the ratio of grown crystal weight to seed weight has not been as high as might be desired. Furthermore, runs of relatively long duration have been required and the available space in the autoclave in which the crystals are grown is not used as efficiently as might be desired. In practice,

## 2

the best results in growing quartz crystals have been obtained heretofore by the use of quartz seed plates having their major opposite faces extending parallel to a minor rhombohedral crystal face. However, a limiting factor in the use of such seed plates is the rapid development of the major rhombohedral faces on crystals grown from seed plates of this type, which cause the tapered shape of the crystal at either end and which decrease the total crystal growth rate, the end result being that much of the grown crystal is not usable for the production of oscillator plates and the like.

In the present invention a significant improvement is obtained in the yield of quartz material usable for piezoelectric plates, both with respect to the crystal seed weight and with respect to the time of the run, as well as with respect to the available autoclave space for growing such crystals.

In accordance with the present invention, the limitations on growth imposed by the primary prism faces and the major rhombohedral faces are avoided to a considerable extent by the use of an elongated quartz seed body whose major faces are inclined at substantial angles to all of the primary prism faces, as well as at substantial angles to all of the major rhombohedral faces. Preferably, the length of the seed body and the period of crystal growth are so chosen that the total crystal growth in any direction on the seed is considerably less than the original seed length. Because of these factors, the major rhombohedral faces and the primary prism faces develop only to a moderate extent in the growing period involved and do not unduly detract from the rate of crystal growth during this period. In addition, the present invention takes advantage of the inherent characteristic of quartz, in the predetermined chemical and physical environments in which quartz crystal growth has been carried on successfully, not to grow to any significant extent outward from its primary prism faces by using an elongated narrow quartz seed body whose length essentially determines the cross-sectional size to which the quartz crystal may grow and whose orientation with respect to the crystallographic axes determines the shape to which the crystal may grow.

Preferably, in the process of the present invention there is employed a crystal seed body elongated in the direction of a crystallographic Y-axis and having a width and thickness much smaller than its length, such as in the ratio of 1 to 20 or more. One practical embodiment employs a seed body of rectangular cross-section, having its elongated narrow major faces extending perpendicular to a crystallographic X-axis and to the crystallographic Z-axis, although different cross-sectional shapes might be used without departing from the spirit and scope of the present invention.

Accordingly, it is an object of the present invention to provide a novel method of growing single crystals of quartz which results in an improved yield of usable crystal material with respect to the crystal seed material required.

Another object of this invention is to provide a novel method of growing single crystals of quartz which results in an improved yield of usable crystal material with respect to the available autoclave capacity.

It is also an object of this invention to provide a novel method of growing single crystals of quartz which results in a greater amount of usable crystal material per unit of run time.

A further object of this invention is to provide a novel method of growing a quartz single crystal in which the growth of usable crystal material takes place rapidly and the decrease in total crystal growth rate resulting from the formation of the major rhombohedral crystal faces is less serious than in the previous methods of quartz synthesis.

Another object of this invention is to provide a novel

method of growing a quartz single crystal which employs a lighter, thinner seed body than required heretofore.

Other and further objects and advantages of the present invention will be apparent from the following description of the preferred embodiment thereof, disclosed in detail in the following description referring to the accompanying drawings.

In the following discussion the standards adopted in the "Standards on Piezoelectric Crystals" (1949) of the Institute of Radio Engineers, set forth in the Proceedings of the I.R.E., vol. 37, pp. 1378-1395, are followed.

In the drawings:

Figure 1 is a perspective view showing an idealized full grown large natural single crystal of quartz of the left-handed variety and showing the orientation of the present quartz seed with respect thereto;

Figure 2 is a transverse cross-section through the middle of the crystal of Fig. 1 and showing the orientation of the present quartz seed;

Figure 3 is an enlarged perspective view of a quartz crystal bar grown in accordance with the present invention;

Figure 4 is a top view, on a reduced scale, of the quartz crystal bar of Fig. 3; and

Figure 5 is a perspective view of the Fig. 3 crystal (on a smaller scale) with the tapered ends of the crystal removed and showing the manner in which oscillator plates may be cut from the crystal.

Referring to Fig. 1, there is shown an idealized natural crystal 10 of left-handed quartz. As is well understood, this crystal is elongated in the direction of the crystallographic Z-axis. At its middle the crystal is bounded by the six primary prism faces 11-16 characterized in crystallography by their Miller index {10̄0}. These primary prism faces extend parallel to the crystallographic Z-axis, which is the direction of natural elongation of quartz. Each of these prism faces is intersected by a pair of neighboring primary prism faces, each inclined at 60° thereto. At one end, in the direction of the crystallographic Z-axis, there are three intersecting major rhombohedral faces, identified by the reference numerals 17, 18 and 19 in Fig. 1. The Miller index for these major rhombohedral faces, as well as for their counterparts 17', 18' and 19' at the opposite end of the crystal, is {10̄1}. Minor rhombohedral faces 20, 21, 22 and 20', 21', 22' of Miller index {01̄1} are located between the major rhombohedral faces. Fig. 1 shows certain additional faces, known as the trigonal bipyramidal and trigonal trapezohedron faces, which sometimes occur in natural quartz crystals but which are not important for an understanding of the present invention.

As shown in Fig. 1, the elongated crystal seed 40 employed in the present process has its length extending in a plane perpendicular to the crystallographic Z-axis (which is the direction of elongation of the crystal) and the crystal seed is elongated in the direction of a crystallographic Y-axis (perpendicular to a pair of parallel opposite primary prism faces, such as 13 and 16) and small in either direction perpendicular to the Y axis. Since the length of the crystal seed extends in the direction of the Y crystallographic axis, the seed is termed a "Y-bar seed." As shown in Fig. 2, the long dimension of the crystal seed 40 extends at 30° to the  $a_1$  crystal axis, at 30° to the  $a_2$  crystal axis, and at 90° to the  $a_3$  crystal axis, these axes being crystallographically equivalent X axes. It will be evident that with any other orientation of the crystal seed perpendicular to the Z crystal axis, the length of the crystal seed would extend at an angle less than 30° with respect to a pair of the prism faces. Accordingly, it may be stated that with the illustrated orientation of the crystal seed the seed length extends at angles to the primary prism faces such that the smallest of these angles is a maximum (30°).

The elongated quartz crystal seed 40 of this orienta-

tion is cut from the mother crystal and is exposed to a predetermined chemical and physical environment which promotes crystal growth on the seed by the deposition of quartz from a transfer medium in which supersaturation of quartz is maintained to cause crystalline growth on the seed. Preferably, the transfer medium is an alkaline aqueous solution in contact with a supply of silica, preferably crystalline quartz, and the quartz seed is exposed to this solution under conditions of elevated temperature and pressure which maintain supersaturation of quartz around the seed to cause crystal growth on the seed. For example, the particular physical and chemical conditions described in the above-mentioned Patent 2,675,303 might be employed. The seed is supported by a suitable holder arrangement (Fig. 3) engaging the seed at or near its opposite ends in the Y-axis direction and permitting unconfined crystal growth on the seed in the directions of the crystallographic X- and Z-axes (perpendicular to the seed length).

From Figs. 1-4 it will be noted that the quartz seed 40 has opposite end faces 13a and 16a which were part of the prism faces 13 and 16 on the mother crystal. These end faces on the seed form substantially the complete primary prism faces of one pair on the crystal bar grown from the seed. In one practical embodiment the seed may be 6 inches long (in the Y-axis direction) and 0.15 inch square in cross-section (parallel to the X- and Z-axes, respectively).

Due to the inherent growth habit of quartz in its nutrient medium, very rapid growth will take place in the direction of the crystallographic Z-axis. This growth will proceed substantially equally on opposite sides of the seed in the Z-axis direction. We have found that quite rapid growth will take place also in the direction of the crystallographic X-axis (the  $a_3$  axis, perpendicular to the length of the seed). However, this growth occurs at a rate about twice as fast on one side of the crystal seed in the X axis direction as on the other side. Rapid growth (but less than the growth rate in the Z- and X-axis directions) takes place on the minor rhombohedral faces. Slow growth takes place on the major rhombohedral faces. Finally, no significant growth occurs on the primary prism faces.

Due to this growth habit, the crystal bar increases rapidly in the Z axis direction on opposite sides of the quartz seed, producing the opposite faces  $Z_{10}$  and  $Z_{11}$  (Fig. 3), which extend perpendicular to the Z axis. Also, the growing crystal bar tends to increase in size rapidly in the X axis direction, producing the opposite faces  $X_{10}$  and  $X_{11}$ , which extend perpendicular to the X axis.

As a result of the rapid growth in the X and Z directions the major rhombohedral faces become larger as the crystal growth proceeds, as do the two pairs of primary prism faces not present on the seed 40.

At the right end of the crystal bar in Fig. 3 the intersecting major rhombohedral faces 17a and 19a are both relatively large. These major rhombohedral faces correspond to the major rhombohedral faces 17 and 19 on the mother quartz (Figure 1). The minor rhombohedral face (corresponding to the minor rhombohedral face 21 on the Fig. 1 mother quartz) which would be expected to appear between the major rhombohedral faces 17a and 19a and the primary prism face 16a (at the end of the crystal seed) has disappeared because of the rapidity with which crystal growth has occurred on it. In like manner, at the opposite end of the seed the crystal bar has developed relatively large major rhombohedral faces 17'a and 19'a, corresponding to the major rhombohedral faces 17' and 19' on the mother quartz of Fig. 1. The minor rhombohedral face which would be expected to appear between these major rhombohedral faces 17'a and 19'a and the primary prism face 13a (at the left end of the seed 40 in Fig. 3) has disappeared because of rapid crystal growth on it.

At the right end of the crystal bar in Fig. 3 the major rhombohedral face  $18'a$ , which corresponds to the major rhombohedral face  $18'$  on the mother crystal of Fig. 1, is considerably smaller in size than the other major rhombohedral faces  $17a$  and  $19a$  at this end of the crystal on the opposite side of the crystal in the Z-axis direction. The minor rhombohedral faces  $20'a$  and  $21'a$  corresponding to the minor rhombohedral faces  $20'$  and  $21'$  on the mother quartz of Fig. 1, border on the major rhombohedral face  $18'a$  at opposite sides thereof.

Similarly, at the left end of the Fig. 3 crystal bar the major rhombohedral face  $18a$ , which corresponds to the major rhombohedral face  $18$  on the Fig. 1 mother crystal, is smaller than the major rhombohedral faces  $17a$  and  $19a$  at this end of the crystal bar on the opposite side of the crystal in the Z-axis direction. The minor rhombohedral faces  $20a$  and  $21a$ , corresponding to the minor rhombohedral faces  $20$  and  $21$  on the mother quartz of Fig. 1, border on the major rhombohedral face  $18a$  on opposite sides thereof.

At the right end of the crystal bar in Fig. 3, the incomplete primary prism face  $15a$  extends away from the end face  $16a$  of the crystal seed (which is also a primary prism face) at an inclination of  $60^\circ$  thereto. Similarly, at the opposite end of the crystal seed the incomplete primary prism face  $14a$  extends (toward the front in Fig. 3) away from the primary prism end face  $13a$  of the crystal seed at an inclination of  $60^\circ$  thereto. The primary prism faces  $15a$  and  $14a$  correspond to the primary prism faces  $15$  and  $14$  on the mother quartz of Fig. 1. These primary prism faces  $15a$  and  $14a$  converge toward each other and would intersect ultimately if full growth of the crystal bar were permitted.

At the right end of the back side of Fig. 3 crystal bar, the incomplete prism face  $11a$  extends away from the primary prism end face  $16a$  on the crystal seed 40 at an inclination of  $60^\circ$  to the latter face. At the opposite end of the crystal seed the incomplete primary prism face  $12a$  extends away from the primary prism end face  $13a$  on the crystal seed at an inclination of  $60^\circ$  to the latter face. These incomplete primary prism faces  $11a$  and  $12a$  correspond to the primary prism faces  $11$  and  $12$  on the mother quartz of Fig. 1. The primary prism faces  $11a$  and  $12a$  converge toward each other and would intersect ultimately if the crystal bar were permitted to grow fully. It will be noted that the primary prism faces  $11a$  and  $12a$  on the back side of the crystal bar in Fig. 3 are more fully developed than the primary faces  $15a$  and  $14a$  at the front side because of the more rapid crystal growth in the X-axis direction on the back side of the crystal seed 40 in Fig. 3.

While the occurrence of crystallographic faces (labelled  $X_{10}$  and  $X_{11}$  in Fig. 3) perpendicular to the X-axis in a grown quartz crystal is believed to be novel and a consequence of the practice of our invention, a difference in growth rate at the opposite ends of such X-axis is in accordance with the well-known polar nature of this axis in quartz. We have found that upon compression in the direction of an X-axis positive charge is developed on the fast-growing end. This finding is of practical value as it enables quartz crystal seeds to be spaced and oriented in an autoclave so as to provide optimum usage of the available space. Correlation between etch figures appearing on a face cut perpendicular to an X-axis of quartz and the electric polarity are well known. For the purpose of orienting our quartz seed, etch figures can therefore also be utilized. On the side of fast growth, the etch pattern produces a characteristic parallelogram when a pin point light source is viewed through the crystal seed bar. From knowledge of the polarity of the X-axis, and the arrangement of major and minor rhombohedral faces around this axis, the handedness of the crystal is determined. Thus, the crystal of Figure 3 is found to be left-handed, and the well-developed front face  $X_{11}$  on the slow growing end of the X-axis has the index {1120}.

If the crystal bar were permitted to grow fully, so that the primary prism faces  $15a$  and  $14a$  would intersect and the primary prism faces  $11a$  and  $12a$  would intersect, as indicated in dotted lines in Fig. 4, then the fully developed prism faces  $16a$ ,  $15a$ ,  $14a$ ,  $13a$ ,  $12a$  and  $11a$  would form a closed hexagonal prism.

It is important to note that the end faces  $16a$  and  $13a$  on the crystal seed do not change in size in the X direction as the crystal growth proceeds, since practically no crystalline growth takes place on these faces and the adjacent prism faces  $15a$ ,  $11a$ , and  $14a$ ,  $12a$ , respectively, because they are primary prism faces. Thus, since the directions in which the incomplete prism faces  $15a$ ,  $11a$ ,  $14a$  and  $12a$  extend away from the primary prism end faces  $16a$  and  $13a$  on the seed are fixed, the size of the crystal bar in the X-axis direction is determined essentially by the length of the crystal seed. Accordingly, it may be considered that crystal growth in the X-axis direction is essentially a filling out of the crystal bar 20 to the cross-sectional size predetermined by the length and the crystallographic orientation of the Y-bar seed.

The major rhombohedral faces  $17a$  and  $19a$  at the right end of the crystal bar in Fig. 3 and the major rhombohedral faces  $17'a$  and  $19'a$  at the left end of this crystal bar impose tapers on the ends of the crystal bar, limiting the growth of usable crystal material in the Z-axis direction.

In order to minimize the waste of crystal material due to the tapers in the Z-axis direction imposed by the major rhombohedral faces and the tapers in the X-axis direction imposed by the primary prism faces which extend away from the ends of the original crystal seed, the crystal preferably should be removed from the nutrient medium long before the crystal has grown fully. The crystal growth should be terminated before the crystal has grown in any direction greater than the length of the original seed. In practice, with a seed having a length of 6 inches in the Y-axis direction, it is desirable to pick the crystal bar after its total growth in the Z-axis direction (its direction of most rapid growth) is of the order of  $\frac{1}{4}$  or less of the seed length. The resultant, partially grown crystal would have a shape approximately that indicated in perspective in Fig. 3 and in full lines in Fig. 4.

By trimming off the tapered ends of this crystal as by cuts along the planes  $c \dots c$  and  $d \dots d$  in Fig. 4, there is produced a block of quartz (Fig. 5) of generally rectangular cross-section, except for minor tapers at certain of its end corners. This block of crystal material would be about 4 inches long in the Y-axis direction, assuming that the original Y bar seed was 6 inches long. Several oscillator plate blanks 41 of an extensively used type, known as the AT cut, may be cut from this crystal block by cutting along spaced, parallel planes disposed at about  $35^\circ$  to the crystallographic Z-axis, as indicated in Fig. 5. With a block of the size specified above, a series of oscillator plate blanks may be cut from the top half of the crystal block shown in Fig. 5 and a series of oscillator plate blanks also may be cut from the bottom half of this crystal block.

With the foregoing arrangement the yield of the crystal material usable for piezoelectric plates, both with respect to the time of the run and with respect to the amount of seed material required, is significantly increased. Due to the small weight of the present crystal seeds and avoidance of much of the unproductive tapered growth which occurs at the final phase of the development of a full grown quartz crystal, a yield of oscillator plate blanks of the order of three or more times that produced by present techniques may be expected, both with respect to the weight of seed material required and with respect to the available autoclave capacity.

Where a crystal is grown in accordance with the present method for the purpose of producing additional Y-bar quartz seeds, rather than oscillator plate blanks, then

it will be preferable to let the crystal grow more fully than the crystal illustrated in Fig. 3.

While in the foregoing description and in the accompanying drawings there has been disclosed a particular preferred embodiment of the present invention, it is to be understood that various modifications, omissions and refinements which depart from the disclosed embodiment may be adopted without departing from the spirit and scope of this invention. For example, the crystal seed might have its length lying in a plane transverse to the Z crystal axis, but not exactly perpendicular thereto. Thus, the length of the crystal seed might extend at an angle as small as 55° to the crystallographic Z-axis, although this will result in a reduced yield and is not considered desirable. Also, the length of the crystal seed might not extend precisely at angles of 90°, 30° and 30° to the respective  $\alpha$ -axes of the crystal (i.e., in the direction of the crystallographic Z-axis). The basic advantages of the present invention would be substantially accomplished even though such minor deviations from the specific preferred embodiment disclosed above are adopted. Accordingly, such variations are considered to fall within the spirit and scope of the present invention.

We claim:

1. A method of growing a quartz single crystal in a predetermined chemical and physical environment which promotes quartz crystal growth and in which environment the quartz crystal tends to have crystal growth on its primary prism faces inhibited, which method comprises the steps of: providing an elongated quartz crystal seed bar having its length extending substantially perpendicular to a crystallographic X-axis and at an angle greater than 55° to the Z axis of the crystal; and exposing said seed bar to a fluid growing medium which provides supersaturation of quartz in the neighborhood of the seed body to cause crystal growth on the seed body.

2. A method of growing a quartz single crystal by the deposition of quartz from a growing medium onto a quartz seed which comprises the steps of: providing an elongated quartz crystal seed bar having its length extending substantially perpendicular to a crystallographic X-axis and substantially perpendicular to the Z-axis of the crystal, said seed bar being small in cross-sectional dimensions perpendicular to its length; and exposing said seed body to a fluid growing medium which provides supersaturation of quartz in the neighborhood of the seed body to cause crystal growth on the seed body.

3. A method of growing a quartz single crystal in a predetermined chemical and physical environment which promotes quartz crystal growth and in which the quartz crystal tends to have substantially no significant growth on its primary prism faces, which method comprises the steps of: providing an elongated quartz crystal seed bar having its length extending in the direction of a Y crystal axis and small in cross-sectional dimensions perpendicular to its length; and exposing said seed bar to said chemical and physical environment to cause crystal growth on the seed bar in the direction of the crystallographic Z-axis, as well as perpendicular to said Z-axis and perpendicular to said Y-axis.

4. A method of growing a quartz single crystal by the deposition of quartz from a transfer medium onto a quartz crystal seed which comprises the steps of: providing an elongated quartz crystal seed bar having its length extending substantially perpendicular to a crystallographic X-axis and at an angle greater than 55° to the crystallographic Z-axis; and exposing said seed to a fluid transfer medium in which a condition of supersaturation of quartz is maintained adjacent the seed to promote crystal growth on the seed.

5. A method of growing a quartz single crystal by the deposition of quartz from an aqueous transfer medium onto a quartz seed which comprises the steps of: providing an elongated quartz crystal seed bar having its length extending substantially perpendicular to the crystallographic Z-axis and substantially perpendicular to a crystallographic X-axis; supporting said seed bar at its ends to permit unconfined crystal growth on the seed bar between its ends in the directions of said X- and Z-axes; and exposing said seed bar, while thus supported, to an aqueous transfer medium in contact with a supply of silica under conditions of elevated temperature and pressure which provide supersaturation of quartz in said medium around the seed bar to promote crystal growth on the seed bar.

6. A method of growing a quartz single crystal by the deposition of quartz from an aqueous solution onto a quartz crystal seed which comprises the steps of: providing an elongated quartz crystal seed bar having its length extending substantially perpendicular to a crystallographic X-axis and at an angle greater than 55° to the crystallographic Z-axis; and exposing said seed bar, while supported for unconfined crystal growth on the seed body between its ends, to an alkaline aqueous solution in contact with a supply of crystalline quartz and under conditions of elevated temperature and pressure which establish supersaturation of quartz in the solution adjacent the seed bar to cause crystal growth on the seed bar.

7. A method of growing a quartz single crystal by the deposition of quartz from an aqueous solution onto a quartz crystal seed which comprises the steps of: providing an elongated quartz crystal seed bar having its length extending substantially parallel to a crystallographic Y-axis and small in cross-sectional dimensions transverse to its length; and exposing said seed bar, while supported at its ends to permit unconfined crystal growth on the seed bar in the directions of the crystallographic X- and Z-axes, under conditions of elevated temperature and pressure to an alkaline aqueous solution in contact with a supply of crystalline quartz and in which solution supersaturation of quartz is maintained to promote crystal growth on the seed bar.

8. A method of growing a quartz single crystal by the transfer of quartz from an aqueous growing solution onto a crystal seed which comprises the steps of: providing an elongated quartz crystal seed bar having its length extending substantially parallel to a crystallographic Y-axis; and exposing said seed bar under growing conditions at elevated temperature and pressure to an aqueous solution in contact with a supply of silica to effect the transfer of quartz onto the seed bar.

#### References Cited in the file of this patent

#### UNITED STATES PATENTS

|            |                 |                |
|------------|-----------------|----------------|
| Re. 19,697 | Kjellgren       | Sept. 10, 1935 |
| 1,906,758  | Kjellgren       | May 2, 1933    |
| 2,309,467  | Mason           | Jan. 26, 1943  |
| 2,468,761  | Kjellgren       | May 3, 1949    |
| 2,508,208  | Wooster         | May 16, 1950   |
| 2,638,408  | Friedman et al. | May 12, 1953   |
| 2,674,520  | Sobek           | Apr. 6, 1954   |
| 2,675,303  | Sobek et al.    | Apr. 13, 1954  |

#### OTHER REFERENCES

Beane et al.: "The Marconi Review," No. 111, vol. XVI, 4th Quarter 1953, pages 141 to 168, Figures 1 and 17.

Thomas et al.: "Faraday Society," Discussion No. 5, 1949, pages 343-344.